



US010481512B2

(12) **United States Patent**  
**Black et al.**

(10) **Patent No.:** **US 10,481,512 B2**  
(45) **Date of Patent:** **\*Nov. 19, 2019**

(54) **PHOTOCOCONDUCTOR HAVING  
PROTECTIVE OVERCOAT LAYER WITH A  
CHARGE TRANSPORT MOLECULE WITH  
FOUR RADICAL POLYMERIZABLE  
HYDROPHILIC FUNCTIONAL GROUPS  
CONTAINING AN OXYGEN ATOM AND  
METHOD OF MAKING THE SAME**

(71) Applicant: **LEXMARK INTERNATIONAL,  
INC.**, Lexington, KY (US)

(72) Inventors: **David Glenn Black**, Broomfield, CO (US); **Mark Thomas Bellino**, Loveland, CO (US); **Weimei Luo**, Louisville, CO (US)

(73) Assignee: **LEXMARK INTERNATIONAL,  
INC.**, Lexington, KY (US)

(\*) Notice: Subject to any disclaimer, the term of this patent is extended or adjusted under 35 U.S.C. 154(b) by 0 days.

This patent is subject to a terminal disclaimer.

(21) Appl. No.: **16/050,321**

(22) Filed: **Jul. 31, 2018**

(65) **Prior Publication Data**

US 2018/0335709 A1 Nov. 22, 2018

**Related U.S. Application Data**

(63) Continuation-in-part of application No. 15/898,687, filed on Feb. 19, 2018, now Pat. No. 10,331,051, (Continued)

(51) **Int. Cl.**  
**G03G 7/00** (2006.01)  
**G03G 5/06** (2006.01)  
(Continued)

(52) **U.S. Cl.**  
CPC ..... **G03G 7/0006** (2013.01); **G03G 5/0607** (2013.01); **G03G 5/071** (2013.01); (Continued)

(58) **Field of Classification Search**  
CPC .. G03G 7/0006; G03G 5/0525; G03G 5/0614; G03G 5/14734  
See application file for complete search history.

(56) **References Cited**

**U.S. PATENT DOCUMENTS**

8,278,017 B2 \* 10/2012 Yu ..... G03G 5/0614  
430/130  
9,034,543 B2 \* 5/2015 Iwadate ..... G03G 5/0618  
430/58.7

(Continued)

*Primary Examiner* — Christopher D Rodee

**ABSTRACT**

An improved organic photoconductor drum used in an electrophotographic image forming device and method to make the same is provided. The organic photoconductor drum contains a protective overcoat. The protective overcoat is prepared from a curable composition including a charge transport molecule containing four radical polymerizable hydrophilic functional groups containing an oxygen atom of the general structure shown below:



where R<sub>1</sub> and R<sub>2</sub> contain a spacer group and a radical polymerizable hydrophilic functional group containing an oxygen atom, R<sub>3</sub> and R<sub>4</sub> are a non-radical polymerizable functional group, and R<sub>5</sub> and R<sub>6</sub> contain a spacer group and (Continued)



a radical polymerizable hydrophilic functional group containing an oxygen atom. The curable composition may also contain at least one curing agent. This organic photoconductor drum has excellent wear resistance without negatively altering the electrophotographic properties, thus protecting the organic photoconductor drum from damage and extending its service life.

- (51) **Int. Cl.**  
*G03G 5/07* (2006.01)  
*G03G 5/147* (2006.01)
- (52) **U.S. Cl.**  
CPC ..... *G03G 5/14786* (2013.01); *G03G 5/14791* (2013.01); *G03G 5/14795* (2013.01)

**7 Claims, 2 Drawing Sheets**

**Related U.S. Application Data**  
which is a continuation of application No. 14/983, 928, filed on Dec. 30, 2015, now Pat. No. 9,927,727, which is a continuation of application No. 14/145, 309, filed on Dec. 31, 2013, now Pat. No. 9,256,143.

- (56) **References Cited**
- U.S. PATENT DOCUMENTS
- |                   |        |               |                               |
|-------------------|--------|---------------|-------------------------------|
| 9,256,143 B2 *    | 2/2016 | Black .....   | <i>G03G 5/0614</i>            |
| 2014/0186758 A1 * | 7/2014 | Bellino ..... | <i>G03G 5/14786</i><br>430/66 |
| 2017/0184984 A1 * | 6/2017 | Black .....   | <i>G03G 5/047</i>             |
- \* cited by examiner



Figure 1



**Figure 2**

## 1

**PHOTOCOCONDUCTOR HAVING  
PROTECTIVE OVERCOAT LAYER WITH A  
CHARGE TRANSPORT MOLECULE WITH  
FOUR RADICAL POLYMERIZABLE  
HYDROPHILIC FUNCTIONAL GROUPS  
CONTAINING AN OXYGEN ATOM AND  
METHOD OF MAKING THE SAME**

**CROSS REFERENCES TO RELATED  
APPLICATIONS**

This application is a continuation in part application of U.S. patent application Ser. No. 15/898,687, filed on Feb. 19, 2018 entitled "METHOD TO MAKE A PHOTOCOCONDUCTOR HAVING AN OVERCOAT WITH TETRAFUNCTIONAL RADICAL POLYMERIZABLE CHARGE TRANSPORT MOLECULE" which is a continuation application of U.S. patent application Ser. No. 14/983,928, filed on Dec. 30, 2015 and now U.S. Pat. No. 9,927,727 and issued Mar. 27, 2018 entitled "METHOD TO MAKE A PHOTOCOCONDUCTOR HAVING AN OVERCOAT WITH TETRAFUNCTIONAL RADICAL POLYMERIZABLE CHARGE TRANSPORT MOLECULE", which is a continuation application of U.S. patent application Ser. No. 14/145,309, now U.S. Pat. No. 9,256,143, filed Dec. 31, 2013 and issued Feb. 9, 2016, entitled "PHOTOCOCONDUCTOR OVERCOAT HAVING TETRAFUNCTIONAL RADICAL POLYMERIZABLE CHARGE TRANSPORT MOLECULE", all of which are assigned to the assignee of the present application.

**BACKGROUND**

**1. Field of the Disclosure**

The present disclosure relates generally to electrophotographic image forming devices, and more particularly to a photoconductor having protective overcoat layer with a charge transport molecule with four radical polymerizable hydrophilic functional groups containing an oxygen atom and method of making the same.

**2. Description of the Related Art**

Organic photoconductor drums have generally replaced inorganic photoconductor drums in electrophotographic image forming device including copiers, facsimiles and laser printers due to their performance and advantages. These advantages include improved optical properties such as having a wide range of light absorbing wavelengths, improved electrical properties such as having high sensitivity and stable chargeability, availability of materials, good manufacturability, low cost, and low toxicity.

While the performance and advantages offered by organic photoconductor drums are significant, inorganic photoconductor drums offer much higher durability. Inorganic photoconductor drums (e.g., amorphous silicon photoconductor drums) are ceramic-based, thus being extremely hard and abrasion resistant. The surface of organic photoconductor drums are typically comprised of a low molecular weight charge transport material, and an inert polymeric binder. Therefore, the failure mechanism for organic photoconductor drums typically arises from mechanical abrasion of the surface layer due to repeated use. Abrasion of photoconductor drum surface may arise from its interaction with print media (e.g. paper), paper dust, or other components of the electrophotographic image forming device.

The abrasion of photoconductor drum surface degrades its electrical properties, such as sensitivity and charging properties. Electrical degradation results in poor image quality,

## 2

such as lower optical density, and background fouling. When a photoconductor drum is locally abraded, images often have black toner bands due to the inability to hold charge in the thinner regions. This black banding often marks the end of the life of the photoconductor drum.

Increasing the life of the photoconductor drum will allow the photoconductor drum to become a permanent part of the electrophotographic image forming device. In other words, the photoconductor drum will no longer be a replaceable unit nor be viewed as a consumable. Photoconductor drums with a life-of-the-printer will allow the printer to operate with lower cost-per-page, more stable image quality, and less waste.

To achieve a long life photoconductor drum, especially with organic photoconductor drum, a protective overcoat layer may be coated onto the surface of the photoconductor drum. While a robust overcoat layer improves the life of photoconductor drums, a suitable overcoat layer is required that does not significantly alter the electrophotographic properties of the photoconductor drum. If the overcoat layer is too electrically insulating, the photoconductor drum will not discharge and will result in a poor latent image. On the other hand, if the overcoat layer is too electrically conducting, then the electrostatic latent image will spread resulting in a blurred image. Thus, a protective overcoat layer that improves life of the photoconductor drum must also allow charge migration to the photoconductor surface for development of the latent image with toner.

Incorporated within overcoats are crosslinkable charge transport molecules. Many prior art overcoats use crosslinkable charge transport molecules having hydrophobic radical polymerizable functional groups. For example, U.S. Pat. No. 9,005,855 to Iwadate teaches that it is desirable for an overcoat to use charge transport molecules having hydrophobic radical polymerizable functional groups as opposed to hydrophilic radical polymerizable functional groups. Iwadate reasons that it is desirable to use a hydrophobic functional group in a charge transport molecule because when hydrophilic or water loving functional groups are used in a charge transport molecule, layer separation in the photoconductor and accordingly deterioration of the efficiency in the charge transport occurs. Additionally, partial moisture absorption naturally caused by using a hydrophilic functional groups in a charge transport molecule leads to a decrease in environmental stability for the photoconductor.

An important feature of the present invention is incorporation of an oxygen atom in the radical polymerizable functional group. The presence of the oxygen atom makes these functional groups hydrophilic by virtue of their ability to hydrogen bond with water. More importantly, radical polymerizable functional groups containing an oxygen atom, such as the acrylate group, methacrylate group, glycidyl ether group and epoxy group, are believed to have higher reactivity towards radical polymerization than olefinic hydrophobic radical polymerizable functional groups such as the styrenic group, the allylic group or the vinylic group. The overcoat of the present invention using charge transport molecules having hydrophilic functional groups as opposed to hydrophobic functional groups, surprisingly leads to a photoconductor having no layer separation, excellent hole mobility and robust mechanical properties.

**SUMMARY**

The present disclosure provides an overcoat layer for an organic photoconductor drum of an electrophotographic

image forming device. The overcoat layer is prepared from a curable composition including a charge transport molecule containing four radical polymerizable hydrophilic functional groups containing an oxygen atom of the general structure exemplified below:



where  $R_1$  and  $R_2$  contain a spacer group and a radical polymerizable hydrophilic group containing an oxygen atom,  $R_3$  and  $R_4$  contain a non-radical polymerizable group, and  $R_5$  and  $R_6$  contain a spacer group and a radical polymerizable hydrophilic group containing an oxygen atom. The curable composition may also contain an optional curing agent.

Also disclosed is a photoconductor drum and method to make the same comprising a support element, a charge generation layer disposed over the support element, a charge transport layer disposed over the charge generation layer, and an overcoat layer disposed over the charge transport layer comprising a curable composition including a charge transport molecule containing four radical polymerizable hydrophilic functional groups containing an oxygen atom as exemplified below:



where  $R_1$  and  $R_2$  contain a spacer group and a radical polymerizable hydrophilic functional group containing an oxygen atom,  $R_3$  and  $R_4$  contain a non-radical polymerizable functional group, and  $R_5$  and  $R_6$  contain a spacer group and a radical polymerizable hydrophilic functional group containing an oxygen atom. The curable composition may also contain an optional curing agent.

#### BRIEF DESCRIPTION OF THE DRAWINGS

The accompanying drawings incorporated in and forming a part of the specification, illustrate several aspects of the present disclosure, and together with the description serve to explain the principles of the present disclosure.

FIG. 1 is a schematic view of an electrophotographic image forming device.

FIG. 2 is a cross-sectional view of a photoconductor drum of the electrophotographic image forming device.

#### DETAILED DESCRIPTION

It is to be understood that the disclosure is not limited in its application to the details of construction and the arrangement of components set forth in the following description or illustrated in the drawings. The disclosure is capable of other embodiments and of being practiced or of being carried out in various ways. Also, it is to be understood that the phraseology and terminology used herein is for the purpose of description and should not be regarded as limiting. The use of "including," "comprising," or "having" and variations thereof herein is meant to encompass the items listed thereafter and equivalents thereof as well as additional items. Further, the terms "a" and "an" herein do not denote a limitation of quantity, but rather denote the presence of at least one of the referenced item.

FIG. 1 illustrates a schematic representation of an example electrophotographic image forming device 100. Image forming device 100 includes a photoconductor drum 101, a charge roll 110, a developer unit 120, and a cleaner unit 130. The electrophotographic printing process is well known in the art and, therefore, is described briefly herein. During a print operation, charge roll 110 charges the surface of photoconductor drum 101. The charged surface of photoconductor drum 101 is then selectively exposed to a laser light source 140 to form an electrostatic latent image on photoconductor drum 101 corresponding to the image being printed. Charged toner from developer unit 120 is picked up by the latent image on photoconductor drum 101 creating a toned image.

Developer unit 120 includes a toner sump 122 having toner particles stored therein and a developer roll 124 that supplies toner from toner sump 122 to photoconductor drum 101. Developer roll 124 is electrically charged and electrostatically attracts the toner particles from toner sump 122. A doctor blade 126 disposed along developer roll 124 provides a substantially uniform layer of toner on developer roll 124 for subsequent transfer to photoconductor drum 101. As developer roll 124 and photoconductor drum 101 rotate, toner particles are electrostatically transferred from developer roll 124 to the latent image on photoconductor drum 101 forming a toned image on the surface of photoconductor drum 101. In one embodiment, developer roll 124 and photoconductor drum 101 rotate in the same rotational direction such that their adjacent surfaces move in opposite directions to facilitate the transfer of toner from developer roll 124 to photoconductor drum 101. A toner adder roll (not shown) may also be provided to supply toner from toner sump 122 to developer roll 124. Further, one or more agitators (not shown) may be provided in toner sump 122 to distribute the toner therein and to break up any clumped toner.

The toned image is then transferred from photoconductor drum 101 to print media 150 (e.g., paper) either directly by photoconductor drum 101 or indirectly by an intermediate transfer member. A fusing unit (not shown) fuses the toner to print media 150. A cleaning blade 132 (or cleaning roll) of cleaner unit 130 removes any residual toner adhering to photoconductor drum 101 after the toner is transferred to print media 150. Waste toner from cleaning blade 132 is held in a waste toner sump 134 in cleaner unit 130. The cleaned surface of photoconductor drum 101 is then ready to be charged again and exposed to laser light source 140 to continue the printing cycle.

The components of image forming device 100 are replaceable as desired. For example, in one embodiment, developer unit 120 is housed in a replaceable unit with photoconductor drum 101, cleaner unit 130 and the main toner supply of image forming device 100. In another embodiment, developer unit 120 is provided with photoconductor drum 101 and cleaner unit 130 in a first replaceable unit while the main toner supply of image forming device 100 is housed in a second replaceable unit. In another embodiment, developer unit 120 is provided with the main toner supply of image forming device 100 in a first replaceable unit and photoconductor drum 101 and cleaner unit 130 are provided in a second replaceable unit. Further, any other combination of replaceable units may be used as desired. In some example embodiment, the photoconductor drum 101 may not be replaced and is a permanent component of the image forming device 100.

FIG. 2 illustrates an example photoconductor drum 101 in more detail. In this example embodiment, the photoconductor drum 101 is an organic photoconductor drum and includes a support element 210, a charge generation layer 220 disposed over the support element 210, a charge transport layer 230 disposed over the charge generation layer 220, and a protective overcoat layer 240 formed as an outermost layer of the photoconductor drum 101. Additional layers may be included between the support element 210, the charge generation layer 220 and the charge transport layer 230, including adhesive and/or coating layers.

The support element 210 as illustrated in FIG. 2 is generally cylindrical. However, the support element 210 may assume other shapes or may be formed into a belt. In one example embodiment, the support element 210 may be formed from a conductive material, such as aluminum, iron, copper, gold, silver, etc. as well as alloys thereof. The surfaces of the support element 210 may be treated, such as by anodizing and/or sealing. In some example embodiment, the support element 210 may be formed from a polymeric material and coated with a conductive coating.

The charge generation layer 220 is designed for the photogeneration of charge carriers. The charge generation layer 220 may include a binder and a charge generation compound. The charge generation compound may be understood as any compound that may generate a charge carrier in response to light. In one example embodiment, the charge generation compound may comprise a pigment being dispersed evenly in one or more types of binders.

The charge transport layer 230 is designed to transport the generated charges. The charge transport layer 230 may include a binder and a charge transport compound. The charge transport compound may be understood as any compound that may contribute to surface charge retention in the dark and to charge transport under light exposure. In one example embodiment, the charge transport compounds may include organic materials capable of accepting and transporting charges.

In an example embodiment, the charge generation layer 220 and the charge transport layer 230 are configured to combine in a single layer. In such configuration, the charge generation compound and charge transport compound are mixed in a single layer. The overcoat layer 240 is designed to protect the photoconductor drum 101 from wear and abrasion without altering the electrophotographic properties, thus extending the service life of the photoconductor drum 101. The overcoat layer 240 has a thickness of about 0.1  $\mu\text{m}$  to about 10  $\mu\text{m}$ . Specifically, the overcoat layer 240 has a thickness of about 1  $\mu\text{m}$  to about 6  $\mu\text{m}$ , and more specifically a thickness of about 3  $\mu\text{m}$  to about 5  $\mu\text{m}$ . The thickness of

the overcoat layer 240 is kept at a range that will not provide adverse effect to the electrophotographic properties of the photoconductor drum 101.

The overcoat layer comprises the cured, or substantially crosslinked, product of a crosslinkable hole transporting material containing four radical polymerizable hydrophilic functional groups containing an oxygen atom. The overcoat layer may further comprise an optional curing agent and an optional non-crosslinkable additive.

The terms "crosslinkable" and "radical polymerizable," and derivatives thereof, may be used interchangeably. "Cured" herein refers to, for example, a state in which the crosslinkable charge transport molecule containing four radical polymerizable hydrophilic groups in the coating solution form a crosslinked or substantially crosslinked product. "Substantially crosslinked" in embodiments refers to, for example, a state in which about 60% to 100% of the charge transport compounds in the overcoat composition, for example about 70% to 100% or about 80% to 100%, are covalently bound in the composition. Curing in the present invention occurs by exposing the curable composition to ionizing electromagnetic radiation of suitable wavelength or by exposure to an electron beam. Crosslinking of the reactive components occurs following application of the overcoat coating composition to the photoconductor.

The following discussion seeks to define the crosslinkable charge transport molecule containing four radical polymerizable hydrophilic groups by describing the fluorene and diphenylamine fragments separately. The crosslinkable charge transport compound of the present invention comprises a nitrogen atom bonded directly to one fluorene group and two phenyl groups.

Fluorene has the following molecular structure:



The fluorene moiety may be fluorene or a fluorene derivative. Fluorene derivatives have the above core structure, with different groups bonded to the core structure. By convention, the carbon atoms are numbered 1-9. The crosslinkable compound of the present invention is substituted in the 9-position with two functional groups comprising a radical polymerizable hydrophilic group. The substituted fluorene group thus has the molecular structure show below:



The substituent's R<sub>1</sub> and R<sub>2</sub> are functional groups containing a spacer group and a radical polymerizable hydrophilic group. The spacer group separates the 9-position of the fluorene ring from the radical polymerizable hydrophilic functional group. The bonds are represented with R<sub>1</sub> coming out of the page, and R<sub>2</sub> going behind the page. In other words, R<sub>1</sub> and R<sub>2</sub> are oriented perpendicular to the plane of

the fluorene group. R<sub>1</sub> and R<sub>2</sub> may be the same or different functional group containing a spacer group and a radical polymerizable hydrophilic group. In an embodiment, R<sub>1</sub> and R<sub>2</sub> are the same functional group containing a spacer group and a radical polymerizable hydrophilic group. The radical polymerizable hydrophilic group is separated from the 9-position of the fluorene ring by a spacer group of at least one carbon. This spacer group may be any branched or unbranched saturated hydrocarbon group having the general formula C<sub>n</sub>H<sub>2n</sub>, wherein n is, for example, a number from 1 to about 100 or more, such as methyl, ethyl, n-propyl, isopropyl, n-butyl, isobutyl, tert-butyl, octyl, decyl, tetradecyl, hexadecyl, eicosyl, tetracosyl, and the like. As used herein, the term spacer group is defined as a C<sub>n</sub>H<sub>2n</sub> group. In an embodiment, the spacer group of R<sub>1</sub> and R<sub>2</sub> is an unbranched alkyl group containing between 1 and about 12 carbon atoms. More specifically, the alkyl group is an unbranched alkyl group containing between 1 and 6 carbon atoms. In an example embodiment, the spacer group of R<sub>1</sub> and R<sub>2</sub> is an ethyl group.

The radical polymerizable hydrophilic group of R<sub>1</sub> and R<sub>2</sub> described herein above is any functional group that contains an oxygen atom, and is capable of undergoing radical polymerization (crosslinking) upon absorption of electromagnetic radiation, or by exposure to an electron beam. The radical polymerizable hydrophilic group containing an oxygen atom may be selected from the group consisting of acrylate group, methacrylate group, glycidyl ether group and epoxy group. In an example embodiment, the radical polymerizable group of R<sub>1</sub> and R<sub>2</sub> is an acrylate group.

The substituted fluorene group thus has the molecular structure shown below:



R<sub>3</sub> and R<sub>4</sub> is different from R<sub>1</sub> and R<sub>2</sub>. R<sub>3</sub> and R<sub>4</sub> both contain a non-radical polymerizable group. The non-radical polymerizable group may be any group without limitation, including H, an alkyl group, an alkoxy group, an aryl group, an aryl alkyl groups, an alcohol group, an alkyl alcohol group and the like. R<sub>3</sub> and R<sub>4</sub> may be covalently bonded to any of the 1-8 positions of the fluorene group. In an example embodiment, R<sub>3</sub> and R<sub>4</sub> are hydrogen atoms. The substituted fluorene group thus has the molecular structure shown below:



The crosslinkable compound of the present invention also comprises two phenyl groups. The phenyl groups further contain substituents R<sub>5</sub> and R<sub>6</sub>. The substituted phenyl groups are exemplified for clarity as the diphenylamine fragment shown below:



The substituents R<sub>5</sub> and R<sub>6</sub> comprise a spacing group and a radical polymerizable hydrophilic functional group. The spacer group separates the phenyl group from the radical polymerizable hydrophilic functional group. The bonds are represented with the bonds for R<sub>5</sub> and R<sub>6</sub> in the same plane as the phenyl group. R<sub>5</sub> and R<sub>6</sub> may be the same or different functional group containing a spacer group and a radical polymerizable hydrophilic group. In an embodiment, R<sub>5</sub> and R<sub>6</sub> are the same functional group containing a spacer group and a radical polymerizable hydrophilic group. The radical polymerizable hydrophilic group is separated from the phenyl group by a spacer group of at least one carbon. This spacer group may be any branched or unbranched saturated hydrocarbon group having the general formula C<sub>n</sub>H<sub>2n</sub>, wherein n is, for example, a number from 1 to about 100 or more, such as methyl, ethyl, n-propyl, isopropyl, n-butyl, isobutyl, tert-butyl, octyl, decyl, tetradecyl, hexadecyl, eicosyl, tetracosyl, and the like. In an embodiment, the spacer group of R<sub>5</sub> and R<sub>6</sub> is an unbranched alkyl group containing between 1 and about 12 carbon atoms. More specifically, the alkyl group is an unbranched alkyl group containing between 1 and 6 carbon atoms. In an example embodiment, the spacer group of R<sub>5</sub> and R<sub>6</sub> is an ethyl group.

The radical polymerizable hydrophilic group of R<sub>5</sub> and R<sub>6</sub> are both located in the para position relative to the nitrogen. The inventors have found that this regiochemistry gives a crosslinkable charge transport compound with electrical properties suitable for a photoconductor of the present invention. The radical polymerizable hydrophilic group of R<sub>5</sub> and R<sub>6</sub> described herein above is any functional group that contains an oxygen atom and is capable of undergoing radical polymerization (crosslinking) upon absorption of electromagnetic radiation, or by exposure to an electron beam. The radical polymerizable group may be selected from the group consisting of acrylate group, methacrylate group, glycidyl ether group and epoxy group. In an example embodiment, the radical polymerizable group is an acrylate group. The radical polymerizable hydrophilic group of R<sub>5</sub> and R<sub>6</sub> may be the same or different from the radical polymerizable hydrophilic group of R<sub>1</sub> and R<sub>2</sub>. In an example embodiment, the radical polymerizable hydrophilic group of R<sub>1</sub>, R<sub>2</sub>, R<sub>5</sub> and R<sub>6</sub> is an acrylate group.

Combining the fluorene and diphenylamine fragments gives the crosslinkable charge transport molecule of the present invention with the molecular structure shown below.



The curable composition of the present invention may also include an optional curing agent. The general purpose of the curing agent is to further improve the abrasion resistance of the overcoat. The curing agent may also improve the adhesion of the cured overcoat to the underlying layer. However, the use of a curing agent in the overcoat is not necessary to result in a photoconductor having excellent hole mobility and robust mechanical properties. In an embodiment, the curing agent, if used, is a urethane resin containing six radical polymerizable functional groups. The radical polymerizable groups may be selected from the group consisting the curable composition of acrylate group, methacrylate group, glycidyl ether group and epoxy group. In another embodiment, the radical polymerizable hydrophilic group is an acrylate. In an example embodiment, the curing agent is a urethane acrylate containing six acrylate groups of the following structure:



and is commercially available from Cytec Industries under the trade name EBECRYL 8301.

The synthesis of urethane acrylates involves reaction of a diisocyanate with pentaerythritol triacrylate in the presence of a catalyst. In a general sense, the choice of isocyanate and/or hydroxy acrylate plays a large role in determining the mechanical and thermal properties of the radically cured material. Curing of urethane acrylates, such as the material described above, creates a 3-dimensionally crosslinked structure. Increasing the crosslink density of the radically cured material is one way to improve the mechanical and thermal properties of the materials. Urethane resins containing six acrylate groups are preferred curing agents for the present invention since crosslink density increases with the number of radical polymerizable functional groups. High crosslink density is known to improve properties such as abrasion and chemical resistance. The crosslinked 3-dimensional network should be homogeneous throughout the cured material, since this improves mechanical and thermal

properties. Homogeneous crosslinking is also important for applications requiring a high degree of optical transparency.

The curable composition comprising a charge transport molecule containing four radical polymerizable hydrophilic functional groups containing an oxygen atom and a curing agent comprising an urethane resin containing six radical polymerizable functional groups exemplifies the overcoat layer 240 with excellent abrasion resistance. In an electro-photographic printer, such as a laser printer, an electrostatic image is created by illuminating a portion of the photoconductor surface in an image-wise manner. The wavelength of light used for this illumination is most typically matched to the absorption max of a charge generation material, such as titanylphthalocyanine. Absorption of light results in creation of an electron-hole pair. Under the influence of a strong electrical field, the electron and hole (radical cation) dissociate and migrate in a field-directed manner. Photoconductors operating in a negative charging manner moves holes to the surface and electrons to ground. The holes discharge the photoconductor surface, thus leading to creation of the latent image. Cured overcoats comprising a charge transport molecule containing four radical polymerizable hydrophilic functional groups containing an oxygen atom provides electrical properties that approach those of the underlying charge transport layer 230. Combining a charge transport molecule containing four radical polymerizable hydrophilic functional groups containing an oxygen atom with a urethane resin containing six radical polymerizable groups provides an overcoat 240 with improved abrasion resistance, along with excellent electrical properties for the photoconductor drum 101.

In one embodiment, the curable composition comprises a combination of a charge transport molecule containing four radical polymerizable hydrophilic functional groups containing an oxygen atom and a curing agent comprising a urethane resin containing six radical polymerizable functional groups. The curable composition includes about 20 to about 80 percent by weight of the charge transport molecule containing four radical polymerizable hydrophilic functional groups containing an oxygen atom, and about 20 to about 80 percent by weight of urethane resin containing six radical polymerizable functional groups. In more particular, the curable composition includes about 40 to about 60 percent by weight of charge transport molecule containing four radical polymerizable hydrophilic functional groups containing an oxygen atom and about 40 to about 60 percent by weight of the urethane resin containing six radical polymerizable functional groups. In another embodiment, the overcoat formulation had the above described charge transport molecules containing four radical polymerizable hydro-

## 11

philic functional groups containing an oxygen atom but no curing agent. The overcoats of the present invention have (1) excellent adhesion to the photoconductor surface, (2) optical transparency and (3) crack free. Ultimately the above described overcoat formulations lead to a photoconductor drum having an 'ultra long life', thereby allowing a consumer to successfully print at least 100,000 pages on their printer before they have to go purchase a replacement photoconductor drum.

Overcoat layers are typically coated in solvent systems designed to solubilize components of the overcoat formulation, while minimizing dissolution of the underlying photoconductor structure. Dissolution of components comprising the underlying photoconductor results in materials with no radical polymerizable functionality entering the overcoat layer. The result is dramatically lower crosslinking density and lower abrasion resistance since the properties of the overcoat layer are optimized by an uninterrupted 3-dimensional network. Ideally, the overcoat layer is distinct from the underlying photoconductor surface. However, the interface between the overcoat and the photoconductor surface often lacks the chemical interactions required for strong adhesion. The overcoats of the present invention have excellent adhesion to the photoconductor surface throughout the print life of the photoconductor. The overcoat must also be optically transparent. Illumination of the photoconductor in an image-wise manner requires that layers not involved in the charge generation process be transparent to the incident light. Additionally, optical transparency is an indicator of material and crosslink homogeneity within the overcoat structure. The overcoats of the present invention have a high degree of optical transparency throughout the print life of the photoconductor. The overcoat must also be crack free. UV or Electron beam cured films often exhibit cracks as a result of unrelieved internal stress. These cracks will manifest immediately in print, and will dramatically decrease the functional life of the overcoat. The overcoats of the present invention are crack free throughout the print life of the photoconductor.

The curable composition may further include a curing agent comprising a monomer or oligomer having at most five radical polymerizable functional groups. The radical polymerizable functional groups of the monomer or oligomer may be selected from the group consisting of acrylate group, methacrylate group, styrenic group, allylic group, vinylic group, glycidyl ether group, epoxy group, or combinations thereof.

Suitable examples of mono-functional monomer or oligomer include, but are not limited to, methyl acrylate, methyl methacrylate, ethyl acrylate, ethyl methacrylate, propyl acrylate, propyl methacrylate, isobornyl acrylate, isobornyl methacrylate, 2-phenoxyethyl acrylate, and lauryl methacrylate.

Suitable examples of di-functional monomer or oligomer include, but are not limited to, diacrylates and dimethacrylates, comprising 1,4-butanediol diacrylate, 1,4-butanediol dimethacrylate, ethylene glycol dimethacrylate, diethylene glycol diacrylate, diethylene glycol dimethacrylate, triethylene glycol diacrylate, triethylene glycol dimethacrylate, 1,3-butylene glycol diacrylate, 1,6-hexanediol diacrylate, 1,6-hexanediol dimethacrylate, 1,12-dodecanediol methacrylate, tripropylene glycol diacrylate, 1,3-butylene glycol dimethacrylate, 1,3-butylene glycol dimethacrylate, cyclohexane dimethanol diacrylate esters, or cyclohexane dimethanol dimethacrylate esters.

Suitable examples of tri-functional monomer or oligomer include, but are not limited to, trimethylolpropane triacry-

## 12

late, trimethylolpropane trimethacrylate, hydroxypropyl acrylate-modified trimethylolpropane triacrylate, ethylene oxide-modified trimethylolpropane triacrylate, propylene oxide-modified trimethylolpropane triacrylate, and caprolactone-modified trimethylolpropane triacrylate. More specifically, the tri-functional monomer or oligomer includes propoxylated (3) trimethylolpropane triacrylate, ethoxylated (6) trimethylolpropane triacrylate, propoxylated (6) trimethylolpropane triacrylate, and ethoxylated (9) trimethylolpropane triacrylate.

Suitable examples of monomers or oligomers having four radical polymerizable functional groups include, but are not limited to, pentaerythritol tetraacrylate, ditrimethylolpropane tetraacrylate, and ethoxylated pentaerythritol tetraacrylate. Suitable examples of monomers or oligomers having five radical polymerizable functional groups include, but are not limited to, pentaacrylate esters and dipentaerythritol pentaacrylate esters.

The curable composition may further include a non-radical polymerizable additive such as a surfactant at an amount equal to or less than about 10 percent by weight of the curable composition. More specifically, the amount of non-radical polymerizable additive is about 0.1 to about 5 percent by weight of the curable composition. The non-radical polymerizable additive may improve coating uniformity of the curable composition.

The curable composition is prepared by mixing the charge transport molecule containing four radical polymerizable hydrophilic groups containing an oxygen atom and optional curing agent in a solvent. The solvent may include organic solvents such as tetrahydrofuran (THF), toluene, alkanes such as hexane, butanone, cyclohexanone and alcohols. The solvent may include a mixture of two or more organic solvents.

The curable composition may be coated on the outermost surface of the photoconductor drum 101 through dipping or spraying. If the curable composition is applied through dip coating, an alcohol is used as the solvent to minimize dissolution of the components of the charge transport layer 230. The alcohol solvent includes isopropanol, methanol, ethanol, butanol, or combinations thereof.

The coated curable composition is then exposed a radiation source of sufficient energy to induce formation of free radicals to initiate the crosslinking reaction. The exposed composition is then post-baked to anneal and relieve stresses in the coating. The radiation source of sufficient energy to induce formation of free radicals is either a UV source, or an electron beam source. If a UV source is used to generate free radicals, the curable composition may contain a photoinitiator.

Specific examples of photo initiators for use under UV cure conditions include acetone or ketal photo polymerization initiators such as diethoxyacetophenone, 2,2-dimethoxy-1,2-diphenylethane-1-one, 1-hydroxy-cyclohexyl-phenyl-ketone, 4-(2-hydroxyethoxy)phenyl-(2-hydroxy-2-propyl)ketone, 2-benzyl-2-dimethylamino-1-(4-molophilinophenyl)butanone-1,2-hydroxy-2-methyl-1-phenylpropane-1-one and 1-phenyl-1,2-propanedion-2-(o-ethoxycarbonyl)oxime; benzoinether photo polymerization initiators such as benzoin, benzoinmethylether, benzoinethylether, benzoinisobutylether and benzoinisopropylether; benzophenone photo polymerization initiators such as benzophenone, 4-hydroxybenzophenone, o-benzoylmethylbenzoate, 2-benzoylnaphthalene, 4-benzoylphenyl, 4-benzoylphenylether, acrylated benzophenone and 1,4-benzoylbenzene; thioxanthone photo polymerization initiators such as 2-isopropylthioxanthone, 2-chlorothioxan-

13

thone, 2,4-dimethylthioxanthone, 2,4-diethylthioxanthone and 2,4-dichlorothioxanthone; phenylglyoxylate photoinitiators such as methylbenzoylformate and other photo polymerization initiators such as ethylanthraquinone, 2,4,6-trimethylbenzoyldiphenylphosphineoxide, 2,4,6-trimethylbenzoyldiphenylethoxyphosphineoxide, bis(2,4,6-trimethylbenzoyl)phenylphosphineoxide, bis(2,4-dimethoxybenzoyl)-2,4,4-trimethylpentylphosphineoxide, methylphenylglyoxyester, 9,10-phenanthrene, acridine compounds, triazine compounds and imidazole compounds. Further, a material having a photo polymerizing effect can be used alone or in combination with the above-mentioned photo polymerization initiators. Specific examples of the materials include triethanolamine, methylmethanol amine, 4-dimethylaminoethylbenzoate, 4-dimethylaminoisoamylbenzoate, ethyl(2-dimethylamino)benzoate and 4,4-dimethylaminobenzophenone. These polymerization initiators can be used alone or in combination. The loading of photoinitiator is between about 0.5 to about 20 parts by weight and more specifically from about 2 to about 10 parts by weight per 100 parts by weight of the curable composition.

Curing the composition by electron beam does not require the presence of a photoinitiator and thus may result in greater crosslink density. In an example embodiment, the radiation source of sufficient energy to induce formation of free radicals is electron beam.

#### Preparation of Example Photoconductor Drum

An Example Photoconductor Drum was formed using an aluminum substrate, a charge generation layer coated onto the aluminum substrate, and a charge transport layer coated on top of the charge generation layer.

The charge generation layer was prepared from a dispersion including type IV titanyl phthalocyanine, polyvinylbutyral, poly(methyl-phenyl)siloxane and polyhydroxystyrene at a weight ratio of 45:27.5:24.75:2.75 in a mixture of 2-butanone and cyclohexanone solvents. The polyvinylbutyral is available under the trade name BX-1 by Sekisui Chemical Co., Ltd. The charge generation dispersion was coated onto the aluminum substrate through dip coating and dried at 100° C. for 15 minutes to form the charge generation layer having a thickness of less than 1 μm, specifically a thickness of about 0.2 μm to about 0.3 μm.

The charge transport layer was prepared from a formulation including terphenyl diamine derivatives and polycarbonate at a weight ratio of 50:50 in a mixed solvent of THF and 1,4-dioxane. The charge transport formulation was coated on top of the charge generation layer and cured at 120° C. for 1 hour to form the charge transport layer having a thickness of about 17 μm to about 19 μm as measured by an eddy current tester.

#### EXAMPLE 1

The inventive overcoat layer of the present invention was prepared from a formulation including EBECRYL 8301 (20 g) and ethanol (80 g) and the crosslinkable charge transport molecule containing four radical polymerizable hydrophilic functional groups containing an oxygen atom (20 g) shown below:

14



The formulation was coated through dip coating on the outer surface of the Example Photoconductor Drum formed as outlined above. The coated layer was then exposed to an electron beam source at an accelerating voltage of 90 kV, a current of 3 mA, and an exposure time of 1.2 seconds. The electron beam cured photoreceptor was then thermally cured at 120° C. for 60 minutes. The cured layer forms the overcoat layer having a thickness of about 4.3 μm as measured by an eddy current tester.

#### COMPARATIVE EXAMPLE 1

An overcoat layer was prepared from a formulation including EBECRYL 8301 (20 g) and ethanol (80 g) and a crosslinkable charge transport molecule containing two radical polymerizable functional groups (20 g) shown below:



The formulation was coated through dip coating on the outer surface of the Example Photoconductor Drum formed as outlined above. The coated layer was then exposed to an electron beam source at an accelerating voltage of 90 kV, a current of 3 mA, and an exposure time of 1.2 seconds. The electron beam cured photoreceptor was then thermally cured at 120° C. for 60 minutes. The cured layer forms the overcoat layer having a thickness of about 4.5 μm as measured by an eddy current tester.

Photoconductor drums Prepared in Example 1 and Comparative Example 1 were installed in an electrophotographic image forming device. The electrophotographic image forming device was then operated at 50 ppm in a four-page and pause run mode. After 40 k prints, the test was stopped and the overcoat thickness loss was determined using an eddy current tester. The initial overcoat thickness (μm), image quality throughout the test, and maximum overcoat thickness loss (μm) after 40 k prints are summarized in Table 1.

TABLE 1

| Example     | Overcoat       |               | Max Overcoat                              | 5  |
|-------------|----------------|---------------|-------------------------------------------|----|
|             | Thickness (μm) | Image Quality | Thickness Loss (μm)<br>(After 40k Prints) |    |
| Example 1   | 4.3            | Excellent     | 0.3                                       |    |
| Comparative | 4.5            | Excellent     | 2.2                                       |    |
| Example 1   |                |               |                                           | 10 |

The overcoat thickness loss from the overcoat of Example 1 is dramatically lower than that of Comparative Example 1. Without wishing to be bound by theory, the inventors believe that there are at least three reasons for the improved abrasion resistance imparted by the crosslinkable charge transport molecule containing four functional groups containing an oxygen atom of the present invention. First, the presence of four radical polymerizable hydrophilic functional groups containing an oxygen atom in the charge transport molecule increases the crosslink density relative to a charge transport molecule having only two radical polymerizable functional groups. Second, the ethyl acrylate groups in the crosslinkable are arrayed such that the groups bonded to the 9-position of the fluorene are perpendicular to the groups bonded to the para position of the two phenyl rings. The inventors believe that this orientation further improves the 3-dimensional crosslinking imparted by the four radical polymerizable hydrophilic functional groups containing an oxygen atom. Third, the spacer group separating the acrylate from the fluorene group and the phenyl groups is an ethyl group. The spacer group separating the four radical polymerizable hydrophilic functional groups containing an oxygen atom from the phenyl group in Comparative Example 1 is a propyl group. The ethyl group allows for still greater crosslink density versus the propyl group by simply removing a methylene fragment.

The foregoing description illustrates various aspects of the present disclosure. It is not intended to be exhaustive. Rather, it is chosen to illustrate the principles of the present disclosure and its practical application to enable one of ordinary skill in the art to utilize the present disclosure, including its various modifications that naturally follow. All modifications and variations are contemplated within the scope of the present disclosure as determined by the appended claims. Relatively apparent modifications include combining one or more features of various embodiments with features of other embodiments.

What is claimed is:

1. An organic photoconductor drum comprising:  
a support element;  
a charge generation layer disposed over the support element;  
a charge transport layer disposed over the charge generation layer; and  
an overcoat layer disposed over the charge transport layer, wherein the overcoat layer includes a cured composition including a charge transport molecule as shown below:



wherein R<sub>1</sub> and R<sub>2</sub> contain a spacer group and a radical polymerizable hydrophilic functional group containing an oxygen atom, R<sub>3</sub> and R<sub>4</sub> are a non-radical polymerizable functional group, and R<sub>5</sub> and R<sub>6</sub> contain a spacer group and a radical polymerizable hydrophilic functional group containing an oxygen atom, and wherein the radical polymerizable hydrophilic functional group containing an oxygen atom of R<sub>1</sub> and R<sub>2</sub> is selected from the group consisting of acrylate group, methacrylate group, glycidyl ether group and epoxy group.

2. The organic photoconductor drum of claim 1, wherein the radical polymerizable functional group containing an oxygen atom of R<sub>1</sub> and R<sub>2</sub> is an acrylate group.

3. The organic photoconductor drum of claim 1, wherein R<sub>3</sub> and R<sub>4</sub> are hydrogen atoms.

4. The organic photoconductor drum of claim 1, wherein the spacer group of R<sub>5</sub> and R<sub>6</sub> is an unbranched alkyl group containing between 1 and about 6 carbon atoms.

5. The organic photoconductor drum of claim 4, wherein the unbranched alkyl group containing between 1 and 6 carbon atoms is an ethyl group.

6. An organic photoconductor drum comprising:  
a support element;  
a charge generation layer disposed over the support element;  
a charge transport layer disposed over the charge generation layer; and  
an overcoat layer disposed over the charge transport layer, wherein the overcoat layer includes a cured composition including a charge transport molecule as shown below:



wherein R<sub>1</sub> and R<sub>2</sub> contain a spacer group and a radical polymerizable hydrophilic functional group containing an oxygen atom, R<sub>3</sub> and R<sub>4</sub> are a non-radical polymerizable functional group, and R<sub>5</sub> and R<sub>6</sub> contain a spacer group and a radical polymerizable hydrophilic functional group containing an oxygen atom, and wherein the radical polymerizable functional group

**17****18**

containing an oxygen atom of R<sub>5</sub> and R<sub>6</sub> is selected from the group consisting of acrylate group, methacrylate group, glycidyl ether group and epoxy group.

7. The organic photoconductor drum of claim 6, wherein the radical polymerizable functional group containing an oxygen atom of R<sub>5</sub> and R<sub>6</sub> is an acrylate group.

\* \* \* \* \*